

1,373,217.

H. WARMAN.  
VITREOUS COATED SHINGLE AND THE LIKE.  
APPLICATION FILED SEPT. 24, 1919.

Patented Mar. 29, 1921.



INVENTOR:

HARRY WARMAN,

By Robert Burns, ATT'Y.

# UNITED STATES PATENT OFFICE.

HARRY WARMAN, OF CLEVELAND, OHIO.

## VITREOUS-COATED SHINGLE AND THE LIKE.

1,373,217.

Specification of Letters Patent. Patented Mar. 29, 1921.

Application filed September 24, 1919. Serial No. 326,030.

To all whom it may concern:

Be it known that I, HARRY WARMAN, a citizen of the United States of America, and a resident of Cleveland, in the county of 5 Cuyahoga, State of Ohio, have invented certain new and useful Improvements in Vitreous-Coated Shingles and the like, of which the following is a specification.

This invention relates to protected sheet 10 metal articles such as roofing shingles, guttering, siding sheets and the like, that are exposed to the weather, and has for its object:

To provide a process and product in which 15 the sheet metal body of a shingle or like article is faced or protected by a weather resisting coating adapted to impart a slate like appearance to the article, and with which a normal flexibility of the article is retained 20 without liability to cracking or seaming the coating.

The accompanying drawing is an enlarged fragmentary section of a coated shingle embodying the present invention.

25 In carrying out the present invention, the sheet metal article after receiving the usual initial treatment has applied to its surface or surfaces a mixture of paste of feldspar, fluorspar, manganese oxid, soda ash, nitrate 30 of soda and borax, preferably in the following proportions:—Feldspar 2 parts, fluorspar  $1\frac{1}{2}$  parts, manganese oxid 1 part, soda ash  $2\frac{1}{2}$  parts, nitrate of soda  $1\frac{1}{2}$  parts and borax  $\frac{1}{2}$  part. The mixture formed into a 35 paste with water is evenly spread on the surface of the article to constitute the primary or ground coating of the same. An exterior or outer surface coating of a granular mineral material, such as ground or crushed 40 slate, quartz, or the like, is evenly spread over the aforesaid primary or ground coating, after which the prepared articles are exposed to a drying operation to remove the

contained moisture in the coating or coatings aforesaid.

The next step in the present process involves the firing of the articles in a suitable kiln or muffle at a temperature approximating 2000° Fahr., the exposure continuing until a very perfect union between said coatings and between the ground coating and the surface of the metal body of the article has been effected, and with the granular nature of said exterior coating still remaining in the outer surface thereof and adapted to afford a granular and very effective surface 50 appearance to the product. The relative thickness of the metal body and of the respective coatings is shown on an enlarged scale in the drawing in which, 1 designates 55 the metal body of the article, 2 the coating of the aforesaid vitreous mixture, and 3 the coating of pulverized slate or the like. A material feature of the present process involves a gradual diminution of the penetration 60 of the one coating into the other. And in that the mineral substances used in said exterior coating can be selected of any desired color and shade, it is possible to produce in a ready manner articles to meet the 65 varied requirements of the trade as to shade, color, etc.

Having thus fully described my said invention what I claim as new and desire to secure by Letters Patent, is:—

75 As an article of manufacture, a sheet metal plate having an inner coating of vitreous material and an exterior coating of crushed slate, said coatings being fused together and to the surface of the articles, with 80 the granular nature of the exterior coating still remaining on the outer surface thereof, substantially as set forth.

Signed at Chicago, Illinois, this 22nd day of September, 1919.

HARRY WARMAN.